

Nov. 26, 1929.

R. E. MARTIN

1,737,318

EXPANSION JOINT

Filed May 25, 1929

*Fig. 1.*



*Fig. 2.*



Inventor

Robert E. Martin (Deceased)  
By Madie Parsons Martin  
Administratrix.

By

*John B. Keenan*  
Attorney

## UNITED STATES PATENT OFFICE

ROBERT E. MARTIN, DECEASED, LATE OF JACKSON, MISSISSIPPI; BY MADIE PARSONS MARTIN, ADMINISTRATRIX, OF JACKSON, MISSISSIPPI

EXPANSION JOINT

Application filed May 25, 1929. Serial No. 365,997.

The present invention relates to the construction of roadways of concrete and like materials, and more particularly to the expansion joints of such roadways.

5 The object of the invention is to provide a convenient and efficient joint unit of improved character, whereby the construction of the roadway is simplified and the strength and durability thereof is enhanced.

10 In constructing roadways or similar structures of concrete or the like, it is necessary to make provision for the expansion and contraction of the concrete under variations of temperature. Unless such provision is made, 15 ordinary changes of temperature cause rapid breaking up and deterioration of the road surface.

It has been proposed heretofore to provide for the expansion and contraction of the concrete by forming expansion joints at intervals in the road. The joints are filled with plastic or yielding material, either poured in liquid form into the joint or inserted therein as a preformed slab.

25 The joints constructed by flowing asphalt or creosote material between the sections of the roadway are laborious and expensive to make and are often unsatisfactory in character. The use of a preformed slab is a distinct improvement but even the joints heretofore constructed in this manner have certain disadvantages.

It has been found that these disadvantages may be overcome and a joint of improved 35 character may be constructed in accordance with the present invention which contemplates an expansion joint embodying a preformed slab or block formed by heating and compressing mechanically disintegrated or exploded wood fibres, the slab being impregnated with asphaltic or creosote material. In general, the impregnating material may be any yielding, water-proofing substance that may be incorporated in the slab or base by an 45 impregnating process. The fibrous base preferably consists of a material commonly known as masonite or masonite fibre, and particularly that variety of masonite having a hard surface portion and a relatively soft core.

50 In the accompanying drawings, Fig. 1 is a

sectional view of a portion of a roadway embodying the invention, and

Fig. 2 is a perspective view of the preformed slab employed in constructing the expansion joint shown in Fig. 1. 55

Referring to the drawings, a portion of a roadway is shown in Fig. 1 embodying sections 1 and 2 of concrete or similar material having an expansion joint 3 interposed therebetween. 60

As shown in Fig. 2, the expansion joint 3 comprises a preformed slab or block of compressed fibrous material, such for example as is known to the trade as masonite or masonite fibre. The preformed slab or block is impregnated with asphaltic or creosote material or the like. Satisfactory results have been obtained with 50-60 penetration asphalt, heated to approximately 450° F., the slab being immersed in the heated bath for 25 or 30 minutes. 70 The process is preferably carried out in such a manner as to insure complete saturation of the slab. 75

The improved results obtained are believed to result primarily from the physical characteristics of the fibrous slab. In forming this slab, wood is converted into fibre by a mechanical disintegration process without removing any substantial amount of the original constituents of the raw material. 80 The process must therefore be distinguished from processes involving a chemical digestion step as in ordinary manufacture of wood pulp. The fibre is preferably prepared by explosion from a gun through a constricted outlet under high pressure, preferably steam pressure of about 250 to 1000 lbs. per sq. in. In a process of this kind, the lignins are retained whereas in processes involving chemical digestion, the lignins are removed or altered in character. Apparently the lignins, under the subsequent steps of the process, serve to produce a binding or cohering of the cellulose fibres whereby the fibrous strip when impregnated, has those characteristics 85 which are desired in an expansion joint. 90

After being fibrated, the woody material is formed into a felted sheet in the usual manner and this sheet is compressed for a sufficient period of time and at such a tempera- 100

ture and pressure as to produce a strong slab of the desired characteristics. While the pressures and temperatures may be varied, it has been found that low pressures produce a slab having a soft core which is particularly advantageous, although relatively high pressures may be employed in some instances. Suitable processes for making masonite fibre are well known in the art, and form the subject-matter of prior patents, such as Nos. 1,663,504 and 1,663,505 granted to W. H. Mason on March 20, 1928.

It has been found that a fibrous slab formed in this manner and impregnated with asphalt or the like is especially adapted for use as an expansion joint of a roadway. The slabs may be cut to the desired size and shipped in quantity to the point of construction and the impregnation of the slabs may be effected when the joints are constructed during the building of the roadway.

What is claimed is:

1. An expansion joint for concrete paving and the like comprising a slab of mechanically disintegrated and compressed wood fibers containing substantially all the constituents of the original raw material, said slab being impregnated with a yielding, water-proofing material.
2. An expansion joint for concrete paving and the like comprising a slab of mechanically disintegrated and compressed wood fibres containing substantially all the constituents of the original raw material, said slab being impregnated with asphaltic material.
3. An expansion joint for concrete paving and the like comprising a slab formed from exploded and compressed fibrous material and impregnated with asphaltic material.
4. An expansion joint for concrete paving and the like comprising a slab of mechanically disintegrated and compressed wood fibres containing substantially all the constituents of the original raw material, said slab having asphalt incorporated therein.
5. The method of constructing an expansion joint comprising the step of impregnating with asphaltic material a slab of exploded woody material which has been compressed until the surface is relatively dense and hard and the core is of lesser density and hardness.
6. The method of constructing an expansion joint comprising the step of impregnating by immersion in asphaltic material of 50-60 penetration for substantially one-half hour a slab of exploded and compressed fibrous material, the asphaltic material being maintained at a temperature of substantially 450° F.

60 MADIE PARSONS MARTIN,  
*Administratrix.*